# EUROPEAN PATENT SPECIFICATION

(11) **EP 2 182 085 B1**
(45) Date of publication and mention of the grant of the patent: **11.10.2017**
(21) Application number: 08777563.1
(22) Date of filing: 18.06.2008
(51) Int. Cl.: C22C 38/00, B21B 1/26, B21B 3/02, C21D 9/46, C22C 38/50, C22C 38/54, C21D 6/00, C21D 8/04, C21D 1/32, C21D 1/673, C22C 38/02, C22C 38/04, C22C 38/42, C22C 38/48

(54) **FERRITIC STAINLESS STEEL PLATE EXCELLENT IN PUNCHABILITY AND PROCESS FOR PRODUCTION OF THE SAME**
PLATTE AUS FERRITISCHEM NICHTROSTENDEM STAHL MIT HERVORRAGENDER STANZBARKEIT UND HERSTELLUNGSVERFAHREN DAFÜR
PLAQUE D'ACIER INOXYDABLE FERRITIQUE PRÉSENTANT UNE EXCELLENTE APTITUDE AU DÉCOUPAGE À LA MATRICE ET SON PROCÉDÉ DE FABRICATION

(30) Priority: 20.08.2007 JP 2007213801
(43) Date of publication of application: 05.05.2010
(73) Proprietor: JFE Steel Corporation, Tokyo, 100-0011 (JP)
(72) Inventor: ISHII, Tomohiro, Tokyo 100-0011 (JP); FUNAKAWA, Yoshimasa, Tokyo 100-0011 (JP); OKADA, Shuji, Tokyo 100-0011 (JP); OHTA, Masayuki, Tokyo 100-0011 (JP)
(74) Representative: Grünecker Patent- und Rechtsanwälte PartG mbB
(86) International application number: PCT/JP2008/061498
(87) International publication number: WO 2009/025125

(56) References cited:
- JP-A- 09 263 912
- JP-A- H08 311 542
- JP-A- 2001 254 153
- JP-A- 2003 213 376
- JP-A- 2004 360 003
- JP-A- 2006 193 771
- US-A- 5 492 575
- US-A1- 2001 003 293

## Description

### Technical Field

The present invention relates to a ferritic stainless steel sheet having a superior punching workability and a method for manufacturing the same.

### Background Art

Since having a superior corrosion resistance and being easily worked, a ferritic stainless steel sheet has been used in various applications, such as architectural materials, transport machines, electric home appliances, and kitchen instruments. In order to manufacture these structures, after a ferritic stainless steel sheet is cut into a predetermined shape, a work, such as forming or welding, is further performed. For cutting of a ferritic stainless steel sheet, a shearing work, which has a high productivity, has been widely used.

In a shearing work, burrs are generated at a cross section of a ferritic stainless steel sheet. In the case in which the height of burrs is large, (a) when a ferritic stainless steel sheet which is cut out is transported to a forming machine (such as a press forming machine), a trouble may arise due to the presence of the burrs, and (b) when welding is performed, since a space may be generated at a burr position of a ferritic stainless steel sheet which is to be welded, for example, burn through may disadvantageously occur. Burrs are not only generated by a shearing work but are also generated by a punching work as shown in Fig, 1B. Hence, development of a punching technique and/or a shearing technique that generates no burrs has been desired.

In the punching work, since a cutting plane is also formed by shearing, the punching work and the shearing work are essentially the same. That is, a generation mechanism of burrs by the punching work is the same as that by the shearing work.

However, heretofore, an investigation to prevent the generation of burrs caused by the punching work and/or the shearing work has not been sufficiently performed, and an investigation to suppress the generation of burrs through an improvement in formability of a steel sheet has been performed.

For example, in Japanese Unexamined Patent Application Publication No. 10-204588, a technique has been disclosed in which recrystallization is facilitated by defining components of a hot-rolled steel sheet and a coiling temperature thereof. According to this technique, in order to improve the formability, the contents of C, P, and S are decreased to decrease precipitates of FeTiP, Ti₄C₂S₂, TiC, and the like. However, in the punching work and/or the shearing work, a large burr is generated.

In Japanese Unexamined Patent Application Publication No. 2002-249857, a technique has been disclosed in which crystal grains of ferrite are coarsened by defining components of a ferritic stainless steel sheet. In this technique, crystal grains of ferrite are coarsened (GSN 5.5 to 8.0) to improve stretch formability of a ferritic stainless steel sheet. However, in the punching work and/or the shearing work, a large burr is liable to be generated.

In Japanese Unexamined Patent Application Publication No. 2002-12955, a technique for improving press formability has been disclosed in which Ti is added, and TiO₂ and Al₂O₃ are suppressed from being precipitated. However, even when the ferritic stainless steel sheet according to this technique is used, in the punching work and/or the shearing work, a large burr is also liable to be generated.

JP 2001 254153 discloses a ferritic stainless steel excellent in weldability which has a layer structure consisting of two or more kinds of compositions containing, by mass, 0.0005 to 0.08% C, 0.01 to 1% Si, 0.01 to 1% Mn, <0.04% P, 0.0001 to 0.01% S, 10 to 25% Cr, 0.0005 to 0.08% N and 0.0005 to 0.01% Mg, furthermore containing one or two kinds of 0.01 to 0.8% Ti and 0.005 to 0.2% A1, and the balance inevitable impurities, also containing one or two kinds of Ti and Al and Mg and containing oxides with the grain size of 0.05 to 5 [mu] m by a distribution density of >=3 pieces/mm² in the steel.

US 5,492,575 discloses a process for producing a thin strip of Cr-stainless steel having high toughness. To produce a thin strip having a high cast strip toughness from a thin cast strip of a Cr-stainless steel containing Nb, Ti, and Al in an amount of 0.05% or more, a process includes the steps of: casting a thin cast strip of a Cr-stainless steel having a thickness of 10 mm or less, the steel containing 13-25 wt % of Cr, 0.05-1 wt % of one or more of Nb, Ti, Al and V in terms of a total amount, 0.03 wt % or less of C, 0.03 wt % or less of N, and 0.3-3.0 wt % of Mo in accordance with need, and having a γp value of 0% or less; hot-rolling the thin cast strip in a temperature range of from 1150 °C to 950 °C at a reduction in thickness of 5 to 50% to form a thin strip; either slowly cooling the thin strip at a rate of 20 °C/sec or less or holding the thin strip for 5 sec or more, in a temperature range of from 1150 °C to 950 °C; and then coiling the thin strip at a temperature lower than 700 DEG C. The γp in % is given by the following formular: 420C+470N+23Ni+9Cu+7Mn-11.5Cr-11.5Si-12 Mo-23V-47Nb-49 Ti-52Al+189 (respective elements in wt %).

A further ferritic stainless steel plate and a method for generating the same is described in US 2001/003293 A1.

An object of the present invention is to provide a ferritic stainless steel sheet which can be processed by a punching work and/or a shearing work without generating burrs and a method for manufacturing the above ferritic stainless steel sheet. Hereinafter, the punching work and the shearing work are collectively called a punching work.

### Disclosure of Invention

The inventors of the present invention carried out an intensive research on causes of burrs generated when a punching work is performed on a ferritic stainless steel sheet. As a result, the following are found.
(A) When a NbTi complex carbonitride is precipitated in grain boundaries of ferrite crystal grains of a ferritic stainless steel sheet, cracks caused by a punching work are likely to be propagated, and as a result, the generation of burrs can be prevented.
(B) When the average ferrite crystal grain size of a ferritic stainless steel sheet measured in accordance with ASTM E 112 is set to 20 µm or less, a NbTi complex carbonitride can be uniformly dispersed.
(C) When the yield ratio of a ferritic stainless steel sheet is set to 0.65 or more, work hardening caused by a punching work is suppressed, and propagation of cracks is facilitated, so that the generation of burrs can be prevented. The present invention was made based on the above findings.

That is, the present invention provides a ferritic stainless steel sheet having a superior punching workability, which comprises: a composition consisting of 0.0030 to 0.012 mass percent of C, 0.13 mass percent or less of Si, 0.25 mass percent or less of Mn, 0.04 mass percent or less of P, 0.005 mass percent or less of S, 0.06 mass percent or less of Al, 0.0030 to 0.012 mass percent of N, 20.5 to 23.5 mass percent of Cr, 0.3 to 0.6 mass percent of Cu, 0.5 mass percent or less of Ni, 0.3 to 0.5 mass percent of Nb, 0.05 to 0.15 mass percent of Ti, and optionally 0.001 mass percent or less of B, 0.1 mass percent or less of Mo, 0.05 mass percent or less of V, 0.01 mass percent or less of Ca; wherein the balance being Fe and inevitable impurities; and a structure in which an average ferrite crystal grain size is 20 µm or less, and a ratio [Nb]/[Ti] of a Nb content to a Ti content contained in a NbTi complex carbonitride present in ferrite crystal grain boundaries is in the range of 1 to 10. In addition, the ferrite crystal grain size is an ASTM nominal grain diameter obtained in accordance with ASTM E 112.

In addition, according to the above ferritic stainless steel sheet of the present invention, the Nb content is 0.3 to 0.45 mass percent, and the Ti content is 0.05 to 0.12 mass percent.

In addition, the present invention provides a method for manufacturing a ferritic stainless steel sheet having a superior punching workability, which comprises: performing hot-rolling of a slab having a composition which consits of 0.0030 to 0.012 mass percent of C, 0.13 mass percent or less of Si, 0.25 mass percent or less of Mn, 0.04 mass percent or less of P, 0.005 mass percent or less of S, 0.06 mass percent or less of Al, 0.0030 to 0.012 mass percent of N, 20.5 to 23.5 mass percent of Cr, 0.3 to 0.6 mass percent of Cu, 0.5 mass percent or less of Ni, 0.3 to 0.5 mass percent of Nb, 0.05 to 0.15 mass percent of Ti, and optionally 0.001 mass percent or less of B, 0.1 mass percent or less of Mo, 0.05 mass percent or less of V, 0.01 mass percent or less of Ca; wherein the balance being Fe and inevitable impurities at a hot-rolling finishing temperature of 900°C or more and at a coiling temperature of 400 to 550°C; performing softening annealing of an obtained hot-rolled steel sheet; then performing pickling; then performing cold rolling; and performing recrystallization annealing of an obtained cold-rolled steel sheet.

In addition, according to the above method for manufacturing a ferritic stainless steel sheet of the present invention, the Nb content is 0.3 to 0.45 mass percent, and the Ti content is 0.05 to 0.12 mass percent.

In addition, according to the method for manufacturing a ferritic stainless steel sheet of the present invention, a slab heating temperature is 1,000°C or less.

According to the present invention, a ferritic stainless steel sheet can be manufactured which can be processed by a punching work without generating large burrs which cause an industrial problem.

### Brief Description of Drawings

[Figs. 1A and 1B] Figs. 1A and 1B show side views of a punching device used in the present invention before and after, respectively, a punching work is performed.
[Fig. 2] Fig. 2 shows a plan view and a side view of a punched-out hole formed by punching out a disc having a diameter of 10 mm.

### Best Modes for Carrying Out the Invention

First, the reasons for limiting components of a ferritic stainless steel sheet of the present invention will be described. In addition, as described above, a punching work and a shearing work are collectively called a punching work.

### C: 0.0030 to 0.012 mass percent

C is an element that binds to Cr, which will be described later, to form a Cr carbide which makes stainless steel sensitive to corrosion. Hence, by addition of Ti and Nb, C is fixed in the form of a NbTi complex carbonitride, and the NbTi complex carbonitride is dispersed and precipitated, so that the generation of burrs caused by a punching work is prevented. When the C content is less than 0.0030 mass percent, the above effect cannot be obtained. On the other hand, when the content is more than 0.012 mass percent, the generation of a Cr carbide cannot be suppressed, and the corrosion resistance is degraded. In addition, since the amount of the NbTi complex carbonitride is increased, and ferrite grains are liable to be expanded and coarsened, burrs are liable to be generated. Hence, the C content is set in the range of 0.0030 to 0.012 mass percent. More preferably, the content is 0.004 to 0.010 mass percent.

### Si: 0.13 mass percent or less

Si is an element that hardens a ferritic stainless steel sheet by solid-solution hardening to degrade the ductility. When the Si content is more than 0.13 mass percent, the ductility of a ferritic stainless steel sheet is considerably degraded. Hence, the Si content is set to 0.13 mass percent or less. More preferably, the content is 0.10 mass percent or less.

### Mn: 0.25 mass percent or less

Mn is an element that degrades the corrosion resistance of a ferritic stainless steel sheet. When the Mn content is more than 0.25 mass percent, in addition to the degradation in corrosion resistance, Mn binds to S which will be described later, and as a result, fine MnS is liable to be generated. MnS is precipitated in grain boundaries of ferrite crystal grains and expands the ferrite crystal grains by hot rolling and/or cold rolling, and as a result, burrs having a large height are generated in a punching work. Hence, the Mn content is set to 0.25 mass percent or less. More preferably, the content is 0.20 mass percent or less.

### P: 0.04 mass percent or less

P is an element that hardens a ferritic stainless steel sheet by solid-solution hardening to degrade the toughness. When the P content is more than 0.04 mass percent, the toughness of a ferritic stainless steel sheet is considerably degraded. Hence, the P content is set to 0.04 mass percent or less. More preferably, the content is 0.03 mass percent or less.

### S: 0.005 mass percent or less

S is an element that binds to Mn or Ti, which will be described later, to form MnS or TiS and disturb equiaxial crystallization of ferrite crystal grains. When the S content is more than 0.005 mass percent, since ferrite crystal grains are considerably expanded, burrs having a large height are generated in a punching work. Hence, the S content is set to 0.005 mass percent or less. More preferably, the content is 0.003 mass percent or less.

### Al: 0.06 mass percent or less

Al is used as a deoxidizing agent in a steelmaking process for forming ferritic stainless steel. In order to obtain the above effect, the content is preferably 0.01 mass percent or more. When the Al content is more than 0.06 mass percent, Al binds to N, and AlN is liable to be generated. AlN expands ferrite crystal grains by hot rolling and/or cold rolling, so that burrs having a large height are generated in a punching work. Hence, the Al content is set to 0.06 mass percent or less. However, when the Al content is less than 0.02 mass percent, the deoxidizing effect cannot be obtained in a steelmaking process. Accordingly, the Al content is preferably in the range of 0.02 to 0.06 mass percent. More preferably, the content is 0.02 to 0.045 mass percent.

### N: 0.0030 to 0.012 mass percent

N generates a NbTi complex carbonitride. When a NbTi complex carbonitride is uniformly dispersed in a ferritic stainless steel sheet, cracks generated by a punching work are likely to be propagated, so that the generation of burrs can be prevented. When the N content is less than 0.0030 mass percent, a sufficient NbTi complex carbonitride amount is not generated. On the other hand, when the content is more than 0.012 mass percent, a Cr nitride is precipitated, so that the corrosion resistance is degraded. Hence, the N content is set in the range of 0.0030 to 0.012 mass percent. More preferably, the content is 0.0040 to 0.010 mass percent.

### Cr: 20.5 to 23.5 mass percent

Cr is an element for forming a passivation film on a surface of a ferritic stainless steel sheet to improve the corrosion resistance. When the Cr content is less than 20.5 mass percent, a superior corrosion resistance to that of a stainless steel containing 18% of Cr, which is an object of the present invention, cannot be obtained. On the other hand, when the content is more than 23.5%, since a hard phase containing Cr and Nb is liable to be precipitated, the workability is degraded, and in addition, recrystallization by annealing after hot rolling (hereinafter referred to as "soft annealing") and/or by annealing after cold rolling (hereinafter referred to as "recrystallization annealing") is disturbed, so that ferrite crystal grains are liable to be expanded in a rolling direction. When the ferrite crystal grains are expanded, burrs having a large height are liable to be generated in a punching work. Hence, the Cr content is set in the range of 20.5 to 23.5 mass percent. More preferably, the content is 20.5 to 22.5 mass percent.

### Cu: 0.3 to 0.6 mass percent

Cu has a function to further improve the corrosion resistance of a ferritic stainless steel sheet containing 20.5 mass percent or more of Cr. When the Cu content is less than 0.3 mass percent, the above effect cannot be obtained. On the other hand, when the content is more than 0.6 mass percent, Cu binds to S, and hence CuS is liable to be generated. CuS expands ferrite crystal grains by hot rolling and/or cold rolling and generates burrs having a large height in a punching work. Hence, the Cu content is set in the range of 0.3 to 0.6 mass percent. More preferably, the content is 0.3 to 0.5 mass percent. Even more preferably, the content is 0.3 to 0.45 mass percent.

### Ni: 0.5 mass percent or less

Ni has a function to further improve the corrosion resistance of a ferritic stainless steel sheet. In order to obtain the above effect, the content is preferably 0.1 mass percent or more. However, when the Ni content is more than 0.5 mass percent, a ferritic stainless steel sheet is hardened, and as a result, the ductility thereof is degraded. Hence, the Ni content is set to 0.5 mass percent or less. More preferably, the content is 0.4 mass percent or less.

### Nb: 0.3 to 0.5 mass percent

Nb has a function to generate a NbTi complex carbonitride in a ferritic stainless steel sheet and to facilitate propagation of cracks generated in a punching work, so that the generation of burrs can be prevented. When the Nb content is less than 0.3 mass percent, a large amount of Cr carbonitride is precipitated, and as a result, the corrosion resistance of a ferritic stainless steel sheet is degraded. On the other hand, when the content is more than 0.5 mass percent, a hard phase containing Cr and Nb is generated, the workability is degraded, and in addition, since the NbTi complex carbonitride is not likely to be generated, burrs having a large height are generated in a punching work. Hence, the Nb content is set in the range of 0.3 to 0.5 mass percent. More preferably, the content is 0.3 to 0.45 mass percent.

### Ti: 0.05 to 0.15 mass percent

Ti has a function to generate a NbTi complex carbonitride in a ferritic stainless steel sheet and to facilitate propagation of cracks generated in a punching work, so that the generation of burrs can be prevented. When the Ti content is less than 0.05 mass percent, the NbTi complex carbonitride is not generated, and a Ti carbonitride and/or a Nb carbonitride is precipitated in ferrite crystal grains. As a result, burrs having a large height are generated in a punching work. On the other hand, when the content is more than 0.15 mass percent, a large amount of TiS is precipitated, equiaxial crystallization of ferrite grains is disturbed, and as a result, burrs having a large height are generated in a punching work. Hence, the Ti content is set in the range of 0.05 to 0.15 mass percent. More preferably, the content is 0.05 to 0.12 mass percent.

The balance other than the components described above contains Fe and inevitable impurities. The amount of the inevitable impurities is preferably decreased as small as possible.

Furthermore, in the ferritic stainless steel sheet of the present invention, at least one selected from the group consisting of B, Mo, V, and Ca is preferably contained.

For example, 0.001 mass percent or less of B, 0.1 mass percent or less of Mo, 0.05 mass percent or less of V, and 0.01 mass percent or less of Ca may be contained.

### B: 0.001 mass percent or less

When a very small amount of B is added, recrystallization nuclei are formed, and as a result, an effect of grain refining crystal grains is obtained. In order to obtain the above effect, the content is preferably 0.0001 mass percent or more. However, when more than 0.001 mass percent of B is added, the workability may be degraded due to steel hardening, and surface defects may occur. Hence, the B content is set to 0.001 mass percent or less.

### Mo: 0.1 mass percent or less

Mo is an element to strengthen a passivation film, facilitate re-passivation after corrosion generation, and improve the corrosion resistance of stainless steel. In order to obtain the above effect, the content is preferably 0.01 mass percent or more. However, when more than 0.1 mass percent is added, the workability, such as press workability, is degraded by solid solution strengthening. Hence, the Mo content is set to 0.1 mass percent or less.

### V: 0.05 mass percent or less

V is an element to improve the corrosion resistance of stainless steel. In order to obtain the above effect, the content is preferably 0.01 mass percent or more. However, when more than 0.05 mass percent is added, steel is hardened, and as a result, the workability is degraded. Hence, the V content is set to 0.05 mass percent or less.

### Ca: 0.01 mass percent or less

Ca is an element to prevent molten steel from adhering to steelmaking devices, such as a nozzle. This effect can be obtained at a content of 0.001 mass percent or more. However, when more than 0.01 mass percent is added, Ca is precipitated in the form, for example, of CaO and CaS in steel. Since these inclusions are easily dissolved in water and increase a local pH, corrosion starts therefrom. Hence, the Ca content is set to 0.01 mass percent or less.

Next, a structure of the ferritic stainless steel sheet of the present invention will be described.

### Average grains size of ferrite crystal grains: 20 µm or less

The size of ferrite crystal grains of a ferritic stainless steel sheet has a significant influence on the height of burrs generated by a punching work. When the grain size is more than 20 µm, deformation of each ferrite crystal grain is increased, and hence, burrs having a large height are liable to be generated. Accordingly, the grain size of ferrite crystal grains is set to 20 µm or less. Incidentally, the ferrite crystal grain size is an ASTM nominal grain diameter obtained in accordance with ASTM E 112.

### Ratio [Nb]/[Ti] between Nb content and Ti content contained in NbTi complex carbonitride: 1 to 10

Cracks caused by a punching work are generated from interfaces between ferrite crystal grains and precipitates present in grain boundaries thereof and are propagated along the grain boundaries. Hence, when a NbTi complex carbonitride is made to be precipitated in grain boundaries of ferrite crystal grains, and when a great number of cracks are made to be generated from the carbonitride and are further made to be combined with each other, cutting can be easily performed. As a result, the generation of burrs in a punching work can be prevented. When the ratio [Nb]/[Ti] between the Nb content and the Ti content contained in the NbTi complex carbonitride is less than 1, adhesion between ferrite grain boundaries and the NbTi complex carbonitride is increased in a punching work, cracks are not likely to be generated, and as a result, the height of burrs is increased. On the other hand, when the ratio [Nb]/[Ti] between the Nb content and the Ti content contained in the NbTi complex carbonitride is more than 10, the NbTi complex carbonitride is particularized, and as a result, cracks are also not likely to be generated at interfaces formed with ferrite grain boundaries. Hence, the ratio [Nb]/[Ti] between the Nb content and the Ti content contained in the NbTi complex carbonitride is set in the range of 1 to 10.

In addition, as a method for measuring the ratio [Nb]/[Ti] between the Nb content and the Ti content contained in the NbTi complex carbonitride, after a thin film is formed from a central portion of a ferritic stainless steel sheet in a thickness direction by a twin jet method, the Nb content [Nb] and the Ti content [Ti] of the NbTi complex carbonitride (inclusions in which a Nb carbonitride and a Ti carbonitride are mixed together on an atomic level, or precipitated inclusions in which one carbonitride functions as precipitation sites and the other carbonitride adheres thereto) precipitated in grain boundaries are measured by a transmission electron microscope, and the [Nb]/[Ti] value is calculated.

Next, mechanical properties of the ferritic stainless steel sheet of the present invention will be described.

### Yield ratio: 0.65 or more

When the yield ratio of a ferritic stainless steel sheet is less than 0.65, since work hardening is liable to occur by a punching work, deformation of each ferrite crystal grain is increased, and hence burrs having a large height are liable to be generated in a punching work. The ferritic stainless steel sheet of the present invention has a yield ratio of 0.65 or more.

Next, a method for manufacturing the ferritic stainless steel sheet of the present invention will be described.

After ferritic stainless steel having predetermined components is formed by melting and is then further formed into a slab, hot rolling (finishing temperature: 900°C or more, coiling temperature: 400 to 550°C) is performed by heating to 1,000°C or more, so that a hot-rolled steel sheet is formed.

### Heating temperature of slab: 1,000°C or more

Carbides and nitrides are once melted by heating a slab, and the finishing temperature and the coiling temperature are defined, so that a NbTi complex carbonitride is made to be precipitated in grain boundaries of ferrite crystal grains. Hence, the heating temperature of the slab is preferably set to 1,000°C or more. In this case, since the slab is deformed at a high temperature, and manufacturing cannot be easily performed, the upper limit of the slab heating temperature is 1,250°C. A more preferable range is 1,050 to 1,200°C.

### Finishing temperature: 900°C or more

When the finishing temperature is less than 900°C, recrystallization is disturbed during hot rolling, so that ferrite crystal grains are expanded in a rolling direction by hot rolling. Hence, burrs having a large height are liable to be generated when a ferritic stainless steel sheet is processed by a punching work. Accordingly, the finishing temperature is set to 900°C or more. In addition, by the reason to prevent seizing with a rolling roll, the upper limit of the finishing temperature is 1,050°C. More preferably, the finishing temperature is in the range of 920 to 1,000°C.

### Coiling temperature: 400 to 550°C

The coiling temperature of a hot-rolled steel sheet has an important function to precipitate a NbTi complex carbonitride in grain boundaries of ferrite crystal grains. When the coiling temperature is less than 400°C, the NbTi complex carbonitride is not precipitated. More preferably, the coiling temperature is in the range of 450 to 530°C.

On the other hand, when the coiling temperature of a hot-rolled steel sheet is more than 550°C, a hard phase containing Nb and Cr is precipitated, and as a result, the toughness is considerably degraded.

Hence, the coiling temperature of a hot-rolled steel sheet is set in the range of 400 to 550°C. When the coiling temperature is in this range, the NbTi complex carbonitride is precipitated in grain boundaries of ferrite crystal grains.

The hot-rolled steel sheet thus obtained is processed by softening annealing and is further processed by pickling. Conditions of the softening annealing and those of the pickling are not particularly limited, and these processes are performed in accordance with known methods. For example, as a preferable condition range for the softening annealing, the temperature is 900 to 1,100°C, and the time is 30 to 180 seconds. Next, cold rolling is performed, so that a cold-rolled steel sheet is obtained. The cold-rolled steel sheet thus obtained is processed by recrystallization annealing, so that a ferritic stainless steel sheet is obtained. Conditions of the cold rolling and those of the recrystallization annealing are not particularly limited, and these processes are performed in accordance with known methods. For example, as a preferable condition range for the recrystallization annealing, the temperature is 900 to 1,100°C, and the time is 30 to 180 seconds. In addition, the cold-rolled steel sheet may be processed by temper rolling. The draft of the temper rolling is preferably in the range of 0.5% to 1.5%.

### Examples

After each ferritic stainless steel having components shown in Table 1 was formed by melting and was further molded into a slab, hot rolling was performed, so that a hot-rolled steel sheet having a thickness of 3 mm was obtained. The conditions of the hot rolling were shown in Table 2. The hot-rolled steel sheet thus obtained was processed by softening annealing (temperature: 900 to 1,100°C, time: 100 to 500 seconds) and was further processed by pickling. Subsequently, cold rolling was performed, so that a cold-rolled steel sheet having a thickness of 0.8 mm was obtained.

The cold-rolled steel sheet thus obtained was processed by recrystallization annealing (temperature: 900 to 1,100°C, time: 100 to 500 seconds) and was further processed by pickling.

After a thin film was formed from a central portion of the ferritic stainless steel sheet thus formed in a thickness direction by a twin jet method, a Nb content [Nb] and a Ti content [Ti] of a NbTi complex carbonitride precipitated in grain boundaries were measured by a transmission electron microscope, and the [Nb]/[Ti] value was calculated. After a structure was exposed by polishing a sheet-thickness cross section parallel to the rolling direction, the ferrite grain size was observed using an optical microscope. Next, 5 line segments each having an actual length of 500 µm were drawn on a photograph in each of a longitudinal direction and a lateral direction, and the number of intersections between the line segments and crystal grain boundaries shown in the photograph was counted. The ASTM nominal grain diameter was obtained in such a way that the total length of the line segments was divided by the number of intersections, and the value obtained thereby was multiplied by 1.13. The results are shown in Table 2. In addition, the measurement of the grain size was performed using one arbitrary viewing field.

In addition, a JIS-No. 13B tensile test piece was formed from the ferritic stainless steel sheet, and a tensile test was performed. The results are shown in Table 2. The tensile test piece was obtained so that a tensile direction was parallel to the rolling direction.

Furthermore, a punching test piece (100 mm by 100 mm) was obtained by cutting the ferritic stainless steel sheet, and a punching test was performed using a punching device shown in Figs. 1A and 1B. After a round hole having a diameter of 10 mm was formed by a punching work at a central portion of the punching test piece, the height of burrs was measured. The results are shown in Table 2. In addition, in Fig. 2, a schematic view of a burr of a punched-out hole formed by punching out a disc having a diameter of 10 mm is shown. The height of the burr of one round hole was measured at 4 points at 90° regular intervals, and the average of the height was obtained therefrom.

Nos. 1 to 5 of Table 2 are examples in each of which the C content was changed. Although the height of the burr of Nos. 2 to 4 which were within the range of the present invention was 50 µm or less, in Nos. 1 and 5 which were out of the range of the present invention, a burr having a height of more than 100 µm was generated.

Nos. 6 to 10 are examples in each of which the Nb content was changed. The height of the burr of Nos. 7 to 9 which were within the range of the present invention was 50 µm or less. In No. 6 in which the Nb content was lower than the range of the present invention, in addition to a low [Nb]/[Ti] value, the grain size of the ferrite crystal grains was large, and the yield ratio was small. Hence, a burr having a height of more than 100 µm was generated. In No. 10 in which the Nb content was higher than the range of the present invention, the ferrite crystal grains were expanded, and a burr having a height of more than 100 µm was generated.

Nos. 11 to 15 are examples in each of which the Ti content was changed. The height of the burr of Nos. 12 to 14 which were within the range of the present invention was 50 µm or less. In No. 11 in which the Ti content was lower than the range of the present invention, the grain size of the ferrite crystal grains was large, and the yield ratio was small. Since the amount of precipitation of the NbTi complex carbonitride was small, a burr having a height of more than 100 µm was generated. In No. 15 in which the Ti content was higher than the range of the present invention, in addition to a low [Nb]/[Ti] value, the grain size of the ferrite crystal grains was large, and the yield ratio was small. Hence, a burr having a height of more than 100 µm was generated.

Nos. 16 to 20 are examples in each of which the N content was changed. The height of the burr of Nos. 17 to 19 which were within the range of the present invention was 50 µm or less. In No. 16 in which the N content was lower than the range of the present invention, since the amount of the NbTi complex carbonitride was small, and the [Nb]/[Ti] value was small, a burr having a height of more than 100 µm was generated. In No. 20 in which the N content was higher than the range of the present invention, in addition to a high [Nb]/[Ti] value, the grain size of the ferrite crystal grains was large, and the yield ratio was small. Hence, a burr having a height of more than 100 µm was generated.

Nos. 21 to 25 are examples in which the conditions of the hot rolling were changed. The height of the burr of Nos. 23 and 24 which were within the range of the present invention was 50 µm or less. In No. 21 in which the finishing temperature and the coiling temperature were out of the range of the present invention, in addition to a low [Nb]/[Ti] value, the grain size of the ferrite crystal grains was large, and the yield ratio was small. Hence, a burr having a height of more than 100 µm was generated. In No. 22 in which the coiling temperature was lower than the range of the present invention, in addition to a low [Nb]/[Ti] value, the grain size of the ferrite crystal grains was large, and the yield ratio was small. Hence, a burr having a height of more than 100 µm was generated. In No. 25 in which the coiling temperature was higher than the range of the present invention, in addition to a high [Nb]/[Ti] value, the grain size of the ferrite crystal grains was large, and the yield ratio was small. Hence, a burr having a height of more than 100 µm was generated.

**TABLE 1**

| No. | COMPONENT (MASS PERCENT) | | | | | | | | | | | |
|---|---|---|---|---|---|---|---|---|---|---|---|---|
| | C | Si | Mn | P | S | Cr | Al | N | Cu | Ni | Nb | Ti |
| 1 | 0.0011 | 0.13 | 0.16 | 0.028 | 0.002 | 20.8 | 0.041 | 0.0077 | 0.39 | 0.13 | 0.38 | 0.08 |
| 2 | 0.0048 | 0.13 | 0.16 | 0.028 | 0.002 | 20.8 | 0.041 | 0.0077 | 0.39 | 0.13 | 0.38 | 0.08 |
| 3 | 0.0085 | 0.13 | 0.16 | 0.028 | 0.003 | 20.8 | 0.041 | 0.0077 | 0.39 | 0.12 | 0.38 | 0.08 |
| 4 | 0.0105 | 0.13 | 0.16 | 0.028 | 0.002 | 20.8 | 0.041 | 0.0077 | 0.39 | 0.14 | 0.38 | 0.08 |
| 5 | 0.0023 | 0.13 | 0.16 | 0.028 | 0.002 | 20.8 | 0.041 | 0.0077 | 0.39 | 0.12 | 0.38 | 0.08 |
| 6 | 0.0066 | 0.06 | 0.21 | 0.032 | 0.001 | 22.3 | 0.024 | 0.0098 | 0.56 | 0.25 | 0.12 | 0.12 |
| 7 | 0.007 | 0.06 | 0.21 | 0.033 | 0.001 | 22.3 | 0.025 | 0.0098 | 0.56 | 0.25 | 0.35 | 0.12 |
| 8 | 0.0068 | 0.06 | 0.21 | 0.031 | 0.001 | 22.3 | 0.024 | 0.0098 | 0.56 | 0.25 | 0.43 | 0.12 |
| 9 | 0.0066 | 0.06 | 0.21 | 0.032 | 0.001 | 22.3 | 0.025 | 0.0098 | 0.56 | 0.25 | 0.48 | 0.12 |
| 10 | 0.0066 | 0.06 | 0.21 | 0.032 | 0.001 | 22.3 | 0.025 | 0.0098 | 0.56 | 0.24 | 0.65 | 0.12 |
| 11 | 0.0102 | 0.08 | 0.13 | 0.018 | 0.004 | 20.5 | 0.055 | 0.0065 | 0.43 | 0.42 | 0.41 | 0.001 |
| 12 | 0.0107 | 0.08 | 0.13 | 0.018 | 0.004 | 20.5 | 0.055 | 0.0065 | 0.43 | 0.42 | 0.41 | 0.07 |
| 13 | 0.0105 | 0.08 | 0.13 | 0.018 | 0.004 | 20.5 | 0.055 | 0.0065 | 0.43 | 0.42 | 0.41 | 0.11 |
| 14 | 0.0108 | 0.08 | 0.13 | 0.018 | 0.004 | 20.5 | 0.055 | 0.0065 | 0.43 | 0.42 | 0.41 | 0.14 |
| 15 | 0.0105 | 0.08 | 0.13 | 0.018 | 0.004 | 20.5 | 0.055 | 0.0065 | 0.43 | 0.42 | 0.41 | 0.26 |
| 16 | 0.0057 | 0.05 | 0.18 | 0.036 | 0.001 | 21.2 | 0.041 | 0.0011 | 0.41 | 0.33 | 0.48 | 0.07 |
| 17 | 0.0059 | 0.05 | 0.18 | 0.035 | 0.001 | 21.2 | 0.041 | 0.0039 | 0.41 | 0.33 | 0.48 | 0.07 |
| 18 | 0.0055 | 0.05 | 0.18 | 0.035 | 0.001 | 21.2 | 0.041 | 0.0066 | 0.41 | 0.33 | 0.48 | 0.07 |
| 19 | 0.0057 | 0.05 | 0.18 | 0.036 | 0.001 | 21.2 | 0.041 | 0.0105 | 0.41 | 0.33 | 0.48 | 0.07 |
| 20 | 0.0023 | 0.08 | 0.18 | 0.035 | 0.001 | 22.0 | 0.041 | 0.0212 | 0.41 | 0.33 | 0.48 | 0.07 |
| 21 | 0.0082 | 0.12 | 0.16 | 0.036 | 0.002 | 23.0 | 0.034 | 0.0107 | 0.34 | 0.44 | 0.34 | 0.09 |
| 22 | 0.0082 | 0.12 | 0.16 | 0.036 | 0.002 | 23.0 | 0.034 | 0.0102 | 0.34 | 0.44 | 0.34 | 0.09 |
| 23 | 0.0085 | 0.12 | 0.16 | 0.036 | 0.002 | 23.0 | 0.034 | 0.0105 | 0.34 | 0.44 | 0.34 | 0.09 |
| 24 | 0.0083 | 0.12 | 0.16 | 0.036 | 0.002 | 23.0 | 0.034 | 0.0107 | 0.34 | 0.44 | 0.34 | 0.09 |
| 25 | 0.0083 | 0.12 | 0.16 | 0.036 | 0.002 | 23.0 | 0.034 | 0.0108 | 0.34 | 0.45 | 0.34 | 0.09 |

**TABLE 2**

| No. | HOT ROLLING | | | NbTi COMPOSITE CARBONITRIDE | FERRITE CRYSTAL GRAINS | MECHANICAL PROPERTIES | | | PUNCHING WORK | REMARKS |
|---|---|---|---|---|---|---|---|---|---|---|
| | HEATING TEMPERATURE (°C) | FINISHING TEMPERATURE (°C) | COILING TEMPERATURE (°C) | [Nb]/[Ti] | GRAIN SIZE (µm) | YIELD RATIO | TENSILE STRENGTH (MPa) | ELONGATION (%) | BURR HEIGHT (µm) | |
| 1 | 1200 | 940 | 420 | 4.4 | 32 | 0.61 | 440 | 36 | 123 | COMPARATIVE EXAMPLE |
| 2 | 1200 | 940 | 420 | 4.4 | 18 | 0.74 | 465 | 35 | 30 | INTENTION EXAMPLE |
| 3 | 1200 | 940 | 420 | 4.4 | 15 | 0.75 | 476 | 34 | 31 | |
| 4 | 1200 | 940 | 420 | 4.4 | 15 | 0.76 | 480 | 32 | 33 | |
| 5 | 1200 | 940 | 420 | 4.4 | 26(EXPANDED GRAIN) | 0.80 | 539 | 26 | 135 | COMPARATIVE EXAMPLE |
| 6 | 1170 | 980 | 400 | 0.9 | 25 | 0.62 | 451 | 34 | 110 | |
| 7 | 1170 | 980 | 400 | 2.7 | 16 | 0.75 | 468 | 34 | 36 | INVENTION EXAMPLE |
| 8 | 1170 | 980 | 400 | 3.3 | 17 | 0.76 | 477 | 33 | 32 | |
| 9 | 1170 | 980 | 400 | 3.7 | 17 | 0.76 | 484 | 33 | 33 | |
| 10 | 1170 | 980 | 400 | 5.0 | 39(EXPANDED GRAIN) | 0.61 | 446 | 35 | 132 | COMPARATIVE EXAMPLE |
| 11 | 1150 | 900 | 400 | - | 26 | 0.63 | 451 | 34 | 105 | |
| 12 | 1150 | 900 | 400 | 5.4 | 18 | 0.76 | 467 | 33 | 33 | INVENTION EXAMPLE |
| 13 | 1150 | 900 | 400 | 3.4 | 17 | 0.77 | 473 | 33 | 34 | |
| 14 | 1150 | 900 | 400 | 2.7 | 16 | 0.77 | 479 | 32 | 35 | |
| 15 | 1150 | 900 | 400 | 0.8 | 28(EXPANDED GRAIN) | 0.61 | 443 | 33 | 122 | COMPARATIVE EXAMPLE |
| 16 | 1180 | 950 | 440 | 0.6 | 17 | 0.75 | 465 | 33 | 131 | |
| 17 | 1180 | 950 | 440 | 6.3 | 16 | 0.74 | 466 | 32 | 45 | INVENTION EXAMPLE |
| 18 | 1180 | 950 | 440 | 6.8 | 15 | 0.75 | 467 | 32 | 37 | |
| 19 | 1180 | 950 | 440 | 7.1 | 15 | 0.76 | 465 | 33 | 34 | |
| 20 | 1180 | 950 | 440 | 1.6 | 26 | 0.63 | 466 | 35 | 139 | COMPARATIVE EXAMPLE |
| 21 | 1160 | 800 | 400 | 0.6 | 45(EXPANDED GRAIN) | 0.64 | 478 | 32 | 144 | |
| 22 | 1160 | 950 | 350 | 0.7 | 36(EXPANDED GRAIN) | 0.66 | 468 | 34 | 137 | |
| 23 | 1160 | 950 | 440 | 3.5 | 16 | 0.73 | 478 | 33 | 42 | INVENTION EXAMPLE |
| 24 | 1160 | 950 | 500 | 3.5 | 17 | 0.72 | 481 | 32 | 43 | |
| 25 | 1160 | 950 | 650 | 2.3 | 25(EXPANDED GRAIN) | 0.65 | 467 | 31 | 146 | COMPARATIVE EXAMPLE |

## Claims

1. A ferritic stainless steel sheet comprising:
a composition which consists of
0.0030 to 0.012 mass percent of C,
0.13 mass percent or less of Si,
0.25 mass percent or less of Mn,
0.04 mass percent or less of P,
0.005 mass percent or less of S,
0.06 mass percent or less of Al,
0.0030 to 0.012 mass percent of N,
20.5 to 23.5 mass percent of Cr,
0.3 to 0.6 mass percent of Cu,
0.5 mass percent or less of Ni,
0.3 to 0.5 mass percent of Nb, 0.05 to 0.15 mass percent of Ti;
and optionally
0.001 mass percent or less of B,
0.1 mass percent or less of Mo,
0.05 mass percent or less of V, 0.01 mass percent or less of Ca;
wherein
the balance being Fe and inevitable impurities;
and a structure in which a ferrite crystal grain size is 20 µm or less, and a ratio [Nb] / [Ti] of a Nb content to a Ti content contained in a NbTi complex carbonitride present in ferrite crystal grain boundaries is in the range of 1 to 10.

2. The ferritic stainless steel sheet according to Claim 1, wherein the Nb content is 0.3 to 0.45 mass percent, and the Ti content is 0.05 to 0.12 mass percent.

3. A method for manufacturing a ferritic stainless steel sheet comprising:
performing hot-rolling of a slab having a composition which consists of
0.0030 to 0.012 mass percent of C,
0.13 mass percent or less of Si,
0.25 mass percent or less of Mn,
0.04 mass percent or less of P,
0.005 mass percent or less of S,
0.06 mass percent or less of Al,
0.0030 to 0.012 mass percent of N,
20.5 to 23.5 mass percent of Cr,
0.3 to 0.6 mass percent of Cu,
0.5 mass percent or less of Ni,
0.3 to 0.5 mass percent of Nb,
0.05 to 0.15 mass percent of Ti;
and optionally
0.001 mass percent or less of B,
0.1 mass percent or less of Mo,
0.05 mass percent or less of V, 0.01 mass percent or less of Ca;
wherein the balance being Fe and inevitable impurities at a hot-rolling finishing temperature of 900°C or more and at a coiling temperature of 400 to 550°C; performing softening annealing of an obtained hot-rolled steel sheet; then performing pickling; then performing cold rolling; and performing recrystallization annealing of an obtained cold-rolled steel sheet.

4. The method for manufacturing the ferritic stainless steel sheet according to Claim 3, wherein the Nb content is 0.3 to 0.45 mass percent, and the Ti content is 0.05 to 0.12 mass percent.

5. The method for manufacturing a ferritic stainless steel sheet according to one of Claims 3 or 4, wherein a slab heating temperature is 1,000°C or less.

## Patentansprüche

1. Ferritisches Edelstahlblech, umfassend:
eine Zusammensetzung bestehend aus
0,0030 bis 0,012 Massenprozent C,
0,13 Massenprozent oder weniger Si,
0,25 Massenprozent oder weniger Mn,
0,04 Massenprozent oder weniger P,
0,005 Massenprozent oder weniger S,
0,06 Massenprozent oder weniger Al,
0,0030 bis 0,012 Massenprozent N,
20,5 bis 23,5 Massenprozent Cr,
0,3 bis 0,6 Massenprozent Cu,
0,5 Massenprozent oder weniger Ni,
0,3 bis 0,5 Massenprozent Nb,
0,05 bis 0,15 Masseprozent Ti;
und optional
0,001 Massenprozent oder weniger B,
0,1 Massenprozent oder weniger Mo,
0,05 Massenprozent oder weniger V,
0,01 Massenprozent oder weniger Ca;
wobei
der Rest Fe und unvermeidliche Verunreinigungen ist;
und eine Struktur, bei der eine Ferritkristallkorngröße 20 µm oder weniger beträgt und ein Verhältnis [Nb] / [Ti] eines Nb-Gehalts zu einem Ti-Gehalt, welcher in einem komplexen NbTi-Carbonitrid enthalten ist, welches in Ferritkristallkorngrenzen vorhanden ist, im Bereich von 1 bis 10 liegt.

2. Ferritisches Edelstahlblech nach Anspruch 1, wobei der Nb-Gehalt 0,3 bis 0,45 Masseprozent beträgt und der Ti-Gehalt 0,05 bis 0,12 Massenprozent beträgt.

3. Verfahren zur Herstellung eines ferritischen Edelstahlblechs, umfassend:
Warmwalzen einer Bramme mit einer Zusammensetzung bestehend aus
0,0030 bis 0,012 Massenprozent C,
0,13 Massenprozent oder weniger Si,
0,25 Massenprozent oder weniger Mn,
0,04 Massenprozent oder weniger P,
0,005 Massenprozent oder weniger S,
0,06 Massenprozent oder weniger Al,
0,0030 bis 0,012 Massenprozent N,
20,5 bis 23,5 Massenprozent Cr,
0,3 bis 0,6 Massenprozent Cu,
0,5 Massenprozent oder weniger Ni,
0,3 bis 0,5 Massenprozent Nb,
0,05 bis 0,15 Massenprozent Ti;
und optional
0,001 Massenprozent oder weniger B,
0,1 Massenprozent oder weniger Mo,
0,05 Massenprozent oder weniger V,
0,01 Massenprozent oder weniger Ca;
wobei der Rest Fe und unvermeidliche Verunreinigungen ist,
bei einer Warmwalzfinishingtemperatur von 900 ° C oder mehr und bei einer Aufwickeltemperatur von 400 bis 550 ° C;
Durchführen eines Erweichungsglühens eines erhaltenen warmgewalzten Stahlblechs; dann Durchführen eines Beizens;
dann Durchführen eines Kaltwalzens; und
Durchführen eines Rekristallisationsglühens eines erhaltenen kaltgewalzten Stahlblechs.

4. Verfahren zur Herstellung eines ferritischen Edelstahlblechs nach Anspruch 3, wobei der Nb-Gehalt 0,3 bis 0,45 Masseprozent beträgt und der Ti-Gehalt 0,05 bis 0,12 Massenprozent beträgt.

5. Verfahren zur Herstellung eines ferritischen Edelstahlblechs nach einem der Ansprüche 3 oder 4, wobei eine Brammenheiztemperatur 1000 °C oder weniger beträgt.

## Revendications

1. Tôle d'acier inoxydable ferritique comprenant :
une composition qui est constituée de
0,0030 à 0,012 pour cent en masse de C,
0,13 pour cent en masse ou moins de Si,
0,25 pour cent en masse ou moins de Mn,
0,04 pour cent en masse ou moins de P,
0,005 pour cent en masse ou moins de S,
0,06 pour cent en masse ou moins d'Al,
0,0030 à 0,012 pour cent en masse de N,
20,5 à 23,5 pour cent en masse de Cr,
0,3 à 0,6 pour cent en masse de Cu,
0,5 pour cent en masse ou moins de Ni,
0,3 à 0,5 pour cent en masse de Nb,
0,05 à 0,15 pour cent en masse de Ti ;
et éventuellement
0,001 pour cent en masse ou moins de B,
0,1 pour cent en masse de Mo,
0,05 pour cent en masse ou moins de V,
0,01 pour cent en masse ou moins de Ca ;
le reste étant constitué de Fe et d'impuretés inévitables ;
et une structure dans laquelle une taille de grain cristallin de ferrite est de 20 µm ou moins, et un rapport [Nb]/[Ti] d'une teneur en Nb sur une teneur en Ti contenues dans un carbonitrure complexe NbTi présent dans les joints des grains cristallins de ferrite est dans la plage de 1 à 10.

2. Tôle d'acier inoxydable ferritique selon la revendication 1, dans laquelle la teneur en Nb est de 0,3 à 0,45 pour cent en masse, et la teneur en Ti est de 0,05 à 0,12 pour cent en masse.

3. Procédé de fabrication d'une tôle d'acier inoxydable ferritique comprenant :
la réalisation d'un laminage à chaud d'une brame ayant une composition qui est constituée de :
0,0030 à 0,012 pour cent en masse de C,
0,13 pour cent en masse ou moins de Si,
0,25 pour cent en masse ou moins de Mn,
0,04 pour cent en masse ou moins de P,
0,005 pour cent en masse ou moins de S,
0,06 pour cent en masse ou moins d'Al,
0,0030 à 0,012 pour cent en masse de N,
20,5 à 23,5 pour cent en masse de Cr,
0,3 à 0,6 pour cent en masse de Cu,
0,5 pour cent en masse ou moins de Ni,
0,3 à 0,5 pour cent en masse de Nb,
0,05 à 0,15 pour cent en masse de Ti ;
et éventuellement
0,001 pour cent en masse ou moins de B,
0,1 pour cent en masse de Mo,
0,05 pour cent en masse ou moins de V,
0,01 pour cent en masse ou moins de Ca ;
le reste étant constitué de Fe et d'impuretés inévitables à une température de finissage de laminage à chaud de 900 °C ou plus et à une température d'enroulement de 400 à 550 °C ; la réalisation d'un recuit d'adoucissement d'une tôle d'acier laminée à chaud obtenue ; puis la réalisation d'un décapage ; puis la réalisation d'un laminage à froid ; puis la réalisation d'un recuit de recristallisation d'une tôle d'acier laminée à froid obtenue.

4. Procédé de fabrication de la tôle d'acier inoxydable ferritique selon la revendication 3, dans lequel la teneur en Nb est de 0,3 à 0,45 pour cent en masse, et la teneur en Ti est de 0,05 à 0,12 pour cent en masse.

5. Procédé de fabrication d'une tôle d'acier inoxydable ferritique selon l'une des revendications 3 ou 4, dans lequel une température de chauffage de brame est de 1 000 °C ou moins.
